# EUROPEAN PATENT SPECIFICATION

(11) **EP 2 843 073 B1**
(45) Date of publication and mention of the grant of the patent: **02.08.2017**
(21) Application number: 13886145.5
(22) Date of filing: 13.06.2013
(51) Int. Cl.: C21D 9/46, C21D 9/50, C21D 1/18, C21D 1/25, C22C 38/00, B22D 11/22, C21D 8/02, C22C 38/02, C22C 38/04, C22C 38/06, C22C 38/08, C22C 38/12, C22C 38/14, C22C 38/16, C22C 38/42, C22C 38/44, C22C 38/46, C22C 38/48, C22C 38/50, C22C 38/54, C22C 38/58

(54) **ULTRAHIGH-TENSILE-STRENGTH STEEL PLATE**
STAHLPLATTE MIT EXTREM HOHER ZUGFESTIGKEIT
TÔLE D'ACIER AVEC TRÈS HAUTE RÉSISTANCE À LA TRACTION

(43) Date of publication of application: 04.03.2015
(73) Proprietor: Nippon Steel & Sumitomo Metal Corporation, Tokyo 100-8071 (JP)
(72) Inventor: WATANABE Yoshiyuki, Tokyo 100-8071 (JP); HARA Takuya, Tokyo 100-8071 (JP); FUJIOKA Masaaki, Tokyo 100-8071 (JP)
(74) Representative: Vossius & Partner Patentanwälte Rechtsanwälte mbB
(86) International application number: PCT/JP2013/066349
(87) International publication number: WO 2014/199488

(56) References cited:
- EP-A1- 1 736 562
- WO-A1-2013/077022
- WO-A1-2013/077022
- JP-A- 2004 100 037
- JP-A- 2006 124 759
- JP-A- 2007 262 508
- JP-A- 2013 095 928

## Description

### [Technical Field of the Invention]

The present invention relates to an ultrahigh tensile strength steel plate for a large welded structure such as an offshore structure or the like which requires a high degree of safety, having excellent weldability and toughness of a heat-affected zone.

### [Related Art]

In recent years, in response to strong global energy demand, the development of marine resources such as oil, natural gas, or the like has been activated. Due to the aforementioned circumstance, an increase in the size of an offshore structure has been pursued due to excavation and production efficiency and severe development conditions. Therefore, there has been a demand for increasing the thickness and strength of steel. In addition, a high degree of safety with regard to against fracture has been required for the offshore structure installed on the sea and excellent weldability and toughness of a heat-affected zone in a steel plate are in demand.

Generally, weldability and toughness of a heat-affected zone of a steel plate tend to deteriorate as the thickness and the strength increase. This is because a large amount of an alloy element which deteriorates the toughness of the heat-affected zone has to be added to ensure strength. While weldability has a wide range of meanings, the weldability generally indicates the hardenability of a heat-affected zone and weld cold crack sensitivity and is indicated by various component parameters such as a carbon equivalent Ceq and a weld crack sensitivity composition P_{CM} in many cases. The greater the amount of the alloy components is, the higher the indices are. Thus, the hardenability of the heat-affected zone and weld cold crack sensitivity increase and generally, the weldability deteriorates. It is known that the toughness of the heat-affected zone is not always consistent with the values of the indices of the weldability but has a high correlation with the values of the indices.

As described above, usually, an increase in the thickness and/or the strength of the steel plate is contradictory to a direction of increasing weldability and toughness of the heat-affected zone and there has been a problem of component design or production technique for attaining the contradictory properties of the steel plate.

As a method of attaining an increase in the thickness and/or strength of a steel plate without deteriorating weldability, that is, without increasing the amount of chemical components more than needed, there is a thermo-mechanical treatment, that is, thermo-mechanical control process (TMCP) and thermal refining treatment (quenching-tempering treatment) for boron (B)-added steel, which are widely known for any person skilled in the art needless to particularly disclose techniques here. However, it is also true that the effect is not sufficient even by the respective methods.

TMCP is for controlling the overall processes of heating-rolling-cooling for producing steel and a water cooling process that is also referred to as accelerated cooling or control cooling is effective to increase the strength of thick material after rolling. However, due to a physical phenomenon called thermal conduction, a sufficient cooling rate cannot be obtained at a thickness center portion of the thick material by water cooling, and it is difficult to ensure an increase in thickness and strength with a low composition.

On the other hand, it is known that since boron (B) used in refined steel having high strength is segregated on prior-austenite grain boundaries in a solid solution state, the hardenability of the steel is significantly increased even with a trace in the order of ppm, and thus, boron is effective to increase the strength. However, this also represents that the hardenability of the heat-affected zone is significantly increased at the same time. In the offshore structure which requires especially a high degree of safety (high fracture toughness of a heat-affected zone), weld heat input is limited being relatively low during the construction and the hardenability is further increased. The hardenability of the heat-affected d zone has a high correlation with the weld cold crack sensitivity and the toughness of the heat-affected zone as described above, and there has been a problem in the unconditional utilization of boron (B). In addition, when high hardenability of boron (B) is utilized, the effect is exhibited only under the presence of boron (B) in a solid solution state, and thus, a component for controlling precipitation of a boron compound, and process control, are necessary. In the combination with TMCP, there has been a case to which findings in the refining treatment cannot be applied as they are. The production by refining treatment, that is, quenching-tempering treatment is disadvantageous in terms of a heat treatment period or cost compared to TMCP. Further, it is fact that non-refining, that is, the attainment of TMCP has been actually socially requested from the viewpoint of environmental load and energy saving in recent years.

Under the circumstances, as steel for an offshore structure having excellent crack tip opening displacement CTOD properties of a welded joint zone having the same thickness and yield strength as those of a main target of the present invention which will be described later, for example, in Patent Document 1, there is disclosed an invention related to Cu-precipitated steel including 0.8% or more of Cu, which is relatively high. However, when a large amount of Cu alone is added, Cu cracking occurs at the time of heating or hot-rolling, and thus, there is a problem of having a difficulty in production.

Patent Document 2 relates to a specific high-strength thick steel plate.

Patent Document 3 relates to a specific high tensile strength steel sheet.

### [Prior Art Document]

### [Patent Document]

[Patent Document 1] Japanese Unexamined Patent Application, First Publication No. 2011-1625
[Patent Document 2] EP 1 736 562 A1
[Patent Document 3] JP 2013-095928 A

### [Disclosure of the Invention]

### [Problems to be Solved by the Invention]

The present invention is made in consideration of the above circumstances and an object thereof is to provide an ultrahigh tensile strength steel plate for a large welded structure such as an offshore structure or the like which requires a high degree of safety, having excellent weldability and toughness of a heat-affected zone.

The main target is a steel plate used for an offshore structure which requires the crack tip opening displacement (CTOD) properties of a welded joint zone with properties of a thickness of 50 mm to 100 mm, a tensile strength of 600 MPa to 700 MPa, a yield strength of 500 MPa to 690 MPa, and the lowest CTOD value of crack tip opening displacement of 0.25 mm or more in a heat-affected zone. It is preferable that the lowest CTOD value is high to ensure sufficient safety against fracture. The usage is not particularly limited and as for the evaluation of the toughness of the heat-affected zone, it is considered that CTOD property evaluation is severer evaluation method compared to Charpy impact properties evaluation, and thus, the steel plate for an offshore structure is set as the main target. Accordingly, it is needless to say that the present invention can be widely applied as a steel plate for welded structures such as vessels, steel frames, bridges, various tanks, or the like.

### [Means for Solving the Problem]

In order to solve various problems that have been pointed out in the related art, on the assumption of TMCP, a method of effectively utilizing boron (B) has been intensively searched and investigated and the inventors found the best method of improving the toughness of the heat-affected zone without deteriorating weldability. The main features are (a) B-N-Ti amount balance optimization for ensuring solid soluted boron (B), (b) C content ultra reduction for alleviating the hardenability of the heat-affected zone by (solid soluted) B, (c) P_{CM} optimization for ensuring the strength, weldability and toughness of the heat-affected zone, (d) Al-free Ti deoxidation for ensuring the toughness of the heat-affected zone, (e) oxide (O) reduction under the Al-free statement for suppressing a coarse oxide, and the like. Since the features are not independent events and have a close relationship among each other, the features are not easily attained at the same time and can be realized by a systematic and precise test conducted by the inventors for the first time and thus, the present invention has been completed.

The gist of the present invention is as follows.
(1) According to a first aspect of the present invention, there is provided a steel plate consisting of, as a chemical composition, by mass%, C: 0.015% to 0.045%, Mn: 1.80% to 2.20%, Cu: 0.40% to 0.70%, Ni: 0.80% to 1.80%, Nb: 0.005% to 0.015%, Mo: 0.05% to 0.25%, Ti: 0.005% to 0.015%, B: 0.0004% to 0.0020%, N: 0.0020% to 0.0060%, O: 0.0015% to 0.0035%, Si: 0.01% to 0.40%, P: 0.008% or less, S: 0.005% or less, Al: 0.0003% to 0.004%, Cr: 0% to 0.30%, V: 0% to 0.06%, Mg: 0% to 0.0050%, and a balance consisting of Fe and unavoidable impurities, wherein a value expressed by a following Expression 1 is more than 2.0, a value expressed by a following Expression 2 is 0% or more, FB expressed by a following Expression 3 is 0.0003% or more, a P_{CM} value which is a weld cracking parameter expressed by a following Expression 4 is 0.18% to 0.23%, a Bp expressed by a following Expression 5 is 0.09% to 0.30% and a number of oxide grains having an equivalent circle diameter of 2 µm or more is 20 particles/mm² or less and a number of Ti oxides having an equivalent circle diameter of 0.05 µm to 0.5 µm is 1.0 × 10³ particles/mm² to 1.0 × 10⁵ particles/mm² at a thickness center portion of a cross section in a thickness direction, $\left[Ni\right] / \left[Cu\right]$ $\left[N\right] - \left[Ti\right] / 3.4$ $FB = \left[B\right] - 0.77 \times \left(\left[N\right]-0.29\times \left(\left[Ti\right]-2\times \left(\left[O\right]-0.89\times \left[Al\right]\right)\right)\right)$ ${P}_{CM} = \left[C\right] + \left[Si\right] / 30 + \left[Mn\right] / 20 + \left[Cu\right] / 20 + \left[Ni\right] / 60 + \left[Cr\right] / 20 + \left[Mo\right] / 15 + \left[V\right] / 10 + 5 \left[B\right]$ $Bp = \left(884\times \left[C\right]\times \left(1-0.3\times {\left[C\right]}^{2}\right)+294\right) \times FB$ here, [C], [Si], [Mn], [Cu], [Ni], [Cr], [Mo], [V], [Ti], [B], [N], [O], and [Al] represent respectively C, Si, Mn, Cu, Ni, Cr, Mo, V, Ti, B, N, O, and Al contents by mass%,
   however, when the term of ([O] - 0.89 × [Al]) in the Expression 3 is 0 or less, the term of ([O] - 0.89 × [Al]) in the Expression 3 is set to 0 to calculate the FB, also, when the term of ([Ti] - 2 × ([O] - 0.89 × [Al])) in the Expression 3 is 0 or less, the term of ([Ti] - 2 × ([O] - 0.89 × [Al])) in the Expression 3 is set to 0 to calculate the FB, further, when the term of ([N] - 0.29 × ([Ti] - 2 × ([O] - 0.89 × [Al]))) in the Expression 3 is 0 or less, the term of ([N] - 0.29 × ([Ti] - 2 × ([O] - 0.89 × [Al]))) in the Expression 3 is set to 0 to calculate the FB, and still further, when FB ≤ 0,FB = 0.
(2) The steel plate according to (1) may further include, as the chemical composition, by mass%, Si: limited to 0.15% or less.
(3) The steel plate according to (1) or (2) may further include, as the chemical composition, by mass%, Mg: limited to less than 0.0003%.
(4) According to the steel plate according to any one of (1) to (3) a thickness may be 50 mm or more and 100 mm or less, a tensile strength may be 600 MPa or more and 700 MPa or less, and a yield strength may be 500 MPa or more and 690 MPa or less.

### [Effects of the Invention]

According to the present invention, it is possible to provide the ultrahigh tensile strength steel having excellent weldability and toughness of the heat-affected zone at a low cost and also possible to further increase safety while the size of a welded structure such as an offshore structure can be increased.

### [Embodiments of the Invention]

Hereinafter, details of the present invention will be described.

An object of the present invention is to provide an ultrahigh tensile strength steel for a large welded structure such as an offshore structure or the like which requires a high degree of safety, having excellent weldability and toughness of the heat-affected zone, and a steel plate having a thickness of 50 mm to 100 mm, a tensile strength of 600 MPa to 700 MPa, a yield strength of 500 MPa to 690 MPa, and the lowest CTOD value of crack tip opening displacement of 0.25 mm or more in the heat-affected zone is a main target.

First, the limited range and the reasons for limitation of the steel components of the ultrahigh tensile strength steel of the present invention will be described. Here, in the following description, % represents mass%.

### C: 0.015% to 0.045%

In the present invention in which high hardenability of B is utilized, it is necessary to suppress an amount of C to be relatively small in order to suppress excessive hardenability of the heat-affected zone. However, when an amount of C is excessively small, an amount of an alloy element for compensating for the strength (tensile strength) has to be increased and thus, economical efficiency is lost. In order to obtain stable strength as the steel that is thick and has a yield strength of 500 MPa to 560 MPa class (which is a strength grade as a steel type and does not indicate an actual yield strength range) as the target of the present invention while an alloy cost is suppressed, the amount of C is limited to 0.015% or more in the present invention. From the viewpoint of economical efficiency, the lower limit thereof may be 0.018%, 0.020%, 0.023% or 0.025%. On the other hand, when the amount of C exceeds 0.045%, the hardness of the heat-affected zone becomes excessive with the effect of B and the toughness of the heat-affected zone is deteriorated. Thus, the upper limit is set to 0.045%. In order to reduce the hardness of the heat-affected zone, the upper limit thereof may be set to 0.042%, 0.040%, 0.037%, or 0.035%.

### Si: 0.01 % to 0.40% or less

Si is unavoidably included in the steel and particularly promotes formation of hard and brittle martensite-austenite (MA) constituent (hereafter, abbreviated to MA) and deteriorates the toughness of the heat-affected zone. Therefore, the smaller the Si is, the more preferable it is. In the present invention in which the amount of C is limited to be relatively small, when Si is included in an amount of up to 0.40%, the MA formation amount is small, and the amount is allowable from the viewpoint of the toughness of the heat-affected zone. However, in consideration of various welding conditions as steel for a welded structure, needless to say, the smaller the amount is, the more preferable it is. The upper limit thereof may be 0.30%, 0.25%, 0.20%, 0.15%, or 0.10% or less.

Si is included to improve the toughness of the base metal of the steel plate or deoxidize the steel, and as necessary, the lower limit thereof is set to 0.01 % or may be 0.02% or 0.03%.

### Mn: 1.80% to 2.20%

Mn is a relatively inexpensive element, but has a great effect to increase the strength and the toughness of the base metal and the heat-affected zone is relatively less adversely affected by Mn. In the present invention in which Al-free Ti deoxidation is performed, it is important to form intragranular ferrite with Ti oxides or the like as nuclei in the heat-affected zone to improve the toughness of the heat-affected zone. However, at this time, Mn also plays an important role. The role is to promote ferrite transformation in such a manner that MnS is precipitated in the Ti oxides to form a Mn depletion region in the vicinity thereof and the transformation temperature is increased higher than that of the matrix. In comprehensive consideration of the strength and toughness of the base metal, the toughness of the heat-affected zone, and further, an alloy cost, the amount of Mn is limited to 1.80% or more in the present invention. The lower limit thereof does not have a critical metallurgical and technical meaning and is limited to make component properties clear within a range in which excellent properties that are targeted in the present invention are exhibited. For the purpose of improving the properties, the lower limit may be set to 1.85% or 1.90%. Mn is an inexpensive element and is attempted to be maximally utilized. However, when the amount of Mn is excessive, center segregation or microsegregation of a continuously cast slab is promoted, and a local embrittled region is formed and thus, it is highly likely to deteriorate the toughness of the base metal or the heat-affected zone. Therefore, the amount of Mn is limited to 2.20% or less. In order to improve the toughness of the base metal or the heat-affected zone, the upper limit thereof may be 2.15% or 2.10%.

### P: 0.008% or less, and S: 0.005% or less

P and S are unavoidably included as impurities and it is preferable that the amount of P and S be small in terms of the toughness of the base metal and the toughness of the HAZ. However, there is limitation in industrial production, and thus, the upper limits of P and S are respectively set to 0.008% and 0.005%. In order to obtain more satisfactory toughness of the HAZ, the upper limit of P may be 0.006%, 0.045%, or 0.004%, and the upper limit of S may be 0.004%, 0.003%, or 0.002%, respectively. P and S are unavoidable impurities and the lower limits of P and S do not need to be defined. If needed, the lower limits of P and S may be 0%.

### Cu: 0.40% to 0.70%

While improving the strength of the base metal, Cu deteriorates the toughness of the base metal and the heat-affected zone relatively less to a small degree and thus, is a useful element. In the ultrahigh tensile strength steel which is the target of the present invention, it is preferable to add 0.40% or more of Cu. In order to improve the strength of the base metal, the lower limit thereof may be 0.45%, 0.50%, or 0.55%. When the amount of Cu exceeds 0.70%, a precipitation hardening phenomenon is exhibited and the material properties of the steel, particularly, the strength is significantly changed in a discontinuous manner. Therefore, in the present invention, the amount of Cu is limited to 0.70% or less as a range in which the strength change is easily controlled in a continuous manner. By limiting the amount of Cu to 0.7% or less, the effect of almost eliminating risk of the occurrence of Cu cracking at the time of hot rolling with the amount of Ni which will be described later is attained. As necessary, the upper limit thereof may be limited to 0.65%, 0.60%, or 0.55%.

### Ni: 0.80% to 1.80%

$\left[Ni\right] / \left[Cu\right] > 2.0$

Ni is known as a highly toughening element and is effective to improve the strength and the toughness of the base metal with less deterioration in the toughness of the heat-affected zone. Therefore, in the ultrahigh tensile strength steel as in the present invention, Ni is a very useful element. Particularly, in the ultralow carbon chemical composition as in the present invention, strength compensation by an alloy element is essential and it is necessary to include at least 0.80% or more of Ni. In order to improve the toughness of the heat-affected zone, the lower limit thereof may be 0.90%, 1.00%, 1.05%, or 1.10%. On the other hand, Ni is an expensive alloy and thus, the content is preferably suppressed to the minimum in which required properties such as strength, toughness, and the like can be obtained. In consideration of the target strength and maximum thickness (100 mm) of the present invention, 1.80% of Ni is required at most and the upper limit thereof is set to 1.80%. However it is needless to say that the upper limit is not a property or metallurgical limit. As necessary, the upper limit thereof may be limited to 1.75%, 1.70%, 1.65%, 1.60%, 1.55%, or 1.50%. In the steel of the present invention including a slightly large amount of Cu as described above, it is effective to include Ni exceeding 2.0 with respect to the amount of Cu to suppress Cu cracking of a cast piece, and Ni is limited to [Ni]/[Cu] > 2.0 in Claim 1.

### Nb: 0.005% to 0.015%

Nb is an effective element to obtain a controlled rolling effect which is effective for structure refinement by expanding an austenite non-recrystallization temperature region to a high temperature region in a rolling process. The structure refinement is an effective method for improving both strength and toughness. At least 0.005% ofNb is necessarily included to reliably obtain the effect As necessary, the lower limit thereof may be 0.006%, 0.007%, or 0.008%. Nb which exhibits such a very useful effect in a base metal increases the hardness of the heat-affected zone to promote MA formation, and thus, is harmful to the toughness. Therefore, the upper limit has to be suppressed to 0.015%. In order to improve the toughness of the heat-affected zone, the upper limit thereof may be 0.013%, 0.011%, or 0.010%.

### Mo: 0.05% to 0.25%

Mo is extremely effective from the viewpoint of improving the strength of the base metal, and is an essential element in the thick high strength steel plate as in the present invention. Particularly, in the present invention in which B is utilized, a higher hardenability improving effect is exhibited by including both Mo and B simultaneously. In order to obtain such excellent effect of Mo, at least 0.05% of Mo is necessarily included. The lower limit thereof may be 0.07%, 0.09%, 0.11%, or 0.13% to reliably exhibit the hardenability improving effect. However, the effect is significant but excessive addition causes a remarkable increase in the hardness and remarkably promotion of MA formation, and thus, it is necessary to limit the amount of Mo to 0.25% or less. In order to suppress MA formation, the upper limit thereof may be 0.23%, 0.21%, 0.19%, or 0.17%.

### Ti: 0.005% to 0.015%

$\left[N\right] - \left[Ti\right] / 3.4 \geq 0 %$

The present invention is an Al-free and Ti-deoxidized steel. It is necessary to include at least 0.005% of Ti since the steel needs to be deoxidizes and the microstructure is refined by forming Ti oxides, and forming intragranular ferrite using the Ti oxides as nuclei in the heat-affected zone. In order to improve the toughness of the heat-affected zone, the lower limit thereof may be 0.006% or 0.007%. However, when the content increases and is stoichiometrically excessive with respect to N, it is highly likely to form TiC by excessive Ti after nitride formation and deteriorate the toughness of the heat-affected zone. Thus, the upper limit is set to 0.015%. In addition, at the same time, from the viewpoint of preventing the TiC precipitation as much as possible, the stoichiometrical relationship between Ti and N is limited to [N] - [Ti]/3.4 ≥ 0%, which represents excess N (lack of Ti) in Claim 1. Here, Ti consumption by deoxidization has to be considered exactly, but it is experimentally confirmed that complication is avoided and also, there is no great influence substantially. In order to obtain a value of Expression 2 of 0% or more, the upper limit of Ti may be 0.013%, 0.012%, 0.011%, or 0.010%.

### B: 0.0004% to 0.0020%

$FB = \left[B\right] - 0.77 \times \left(\left[N\right]-0.29\times \left(\left[Ti\right]-2\times \left(\left[O\right]-0.89\times \left[Al\right]\right)\right)\right) \geq 0.0003 %$

B is one of important elements in the present invention. The hardenability improving effect of B is very high and an alloy element can be significantly suppressed by utilizing B. Therefore, it is necessary that the amount of B is at least 0.0004%. As necessary, the lower limit thereof may be 0.0005%, 0.0006%, or 0.0007%. However, it is not sufficient to simply define only the B content. This is because that B has to be in a solid solution state to utilize the hardenability of B. B easily forms nitrides and a stoichiometrical balance between B and N is important. However, Ti has higher nitride forming capacity than B, and thus, considering the fact, B is limited to FB = [B] - 0.77 × ([N] - 0.29 × ([Ti] - 2 × ([O] - 0.89 × [Al]))) ≥ 0.0003% in Claim 1. Even when B is included more than needed, the effect is saturated and thus, the inventors have set the upper limit to 0.0020% as a range that is experimentally confirmed for a range in which the properties of the steel is not adversely affected. However, the value does not need to have critical significance. As necessary, the upper limit thereof may be limited to 0.0018%, 0.0016%, 0.0015%, or 0.0014%.

For the purpose of ensuring B that is present in a solid solution state in the steel (effective B), it has been found that 0.0003% or more of the FB as a parameter indicating the amount of the effective B defined by the Expression 3 is required. The FB may be set to 0.0004% or more, or 0.0005% to more effectively utilize B.

The upper limit of FB = [B] - 0.77 × ([N] - 0.29 × ([Ti] - 2 × ([O] - 0.89 × [Al]))) is not particularly limited, but is naturally limited from the limitation range of each element

However, when the term of ([O] - 0.89 × [Al]) in the Expression 3 is 0 or less, the term of ([O] - 0.89 × [Al]) in the Expression 3 is set to 0 to calculate the FB.

In addition, in the Expression 3, when the term of ([Ti] - 2 × ([O] - 0.89 × [Al])) in the Expression 3 is 0 or less, the term of ([Ti] - 2 × ([O] - 0.89 × [Al])) in the Expression 3 is set to 0 to calculate the FB.

Further, when the term of ([N] - 0.29 × ([Ti] - 2 × ([O] - 0.89 × [Al]))) in the Expression 3 is 0 or less, the term of ([N] - 0.29 × ([Ti] - 2 × ([O] - 0.89 × [Al]))) in the Expression 3 is set to 0 to calculate the FB.

Still further, when FB ≤ 0, FB = 0.

In addition, the Expression 3 is an expression for obtaining the amount of the solid soluted B (the amount of effective B: FB) in the steel obtained from a stoichiometric ratio in consideration of a bonding force strength between the respective elements. The upper limit of the FB does not need to be defined particularly but may be 0.0010%.

As a result of further investigation, it is found that a B parameter Bp which is defined by Expression 5 as a parameter for avoiding an increase the hardness of the HAZ due to B is 0.09% to 0.30%. $Bp = \left(884\times \left[C\right]\times \left(1-0.3\times {\left[C\right]}^{2}\right)+294\right) \times FB$

Here, Bp is an empirical equation derived from the analysis by testing plural pieces of molten steel at an experimental laboratory and is parameterized by (the highest hardness estimated by amount of C) x (FB contribution). As the FB increases, the hardness of the HAZ tends to be increased. Particularly, the CTOD properties are significantly affected as this case. When Bp exceeds 0.30%, the hardness of a fusion line (FL) is remarkably increased in some cases, and thus, it has been found that the Bp is limited to 0.30% or less to satisfy 0.25 mm or more that is the target value of the CTOD properties. As necessary, the upper limit of the Bp may be 0.27% or 0.25%. When the FB is 0.0003% or more in the welded steel according to the embodiment, the Bp has to be 0.09% or more, and thus, Bp of less than 0.09% within a region in which the effect of the solid soluted B targeted in the welded steel according to the embodiment cannot be obtained. Therefore, the Bp is 0.09% or more. As necessary, the lower limit of the Bp may also be 0.12% or 0.15%.

### N: 0.0020% to 0.0060%

N is an element which is unavoidably included in steel production and the reduction of N more than needed increases a load on steel production and is not preferable in terms of industrial production. N rather forms nitrides with the addition of Ti. In addition, the nitrides are stable at a high temperature and thus, have an effect of pinning austenite grain growth coarsening at the time of heating before hot-rolling the steel or in the heat-affected zone that is slightly away from the fusion line. Therefore, it is preferable that 0.0020% or more of N be included. However, when the amount of N is excessive, N is bonded with B to form nitrides as described above, and thus, the hardenability improving effect of B is highly likely to be reduced. From the above-described absolute amount and stoichiometric relationship between B and Ti, the upper limit is naturally limited, but additionally, when the amount of N exceeds 0.0060%, a surface defect occurs at the time of producing a steel piece. Thus, the upper limit is set to 0.0060%. The upper limit is preferably 0.0055% or less, and more preferably 0.005% or less.

### O: 0.0015% to 0.0035%

From the formability of the Ti oxides as nuclei for forming intragranular ferrite in the heat-affected zone, 0.0015% or more of O is required. However, when the amount of O is excessive, the size or the number of the oxides excessively increases and the oxides are highly likely to act as a starting point of brittle fracture. As a result, the toughness is deteriorated. Thus, it is necessary that the upper limit be limited to 0.0035%. In order to obtain more satisfactory stable toughness of the heat-affected zone, the amount of O is preferably 0.0030% or less, and more preferably 0.0028% or less, or 0.0025% or less.

### Al: 0.0003% to 0.004%

In the present invention of the Al-free and Ti deoxidation steel, Al is one of unavoidable impurities. The reason for limiting the upper limit in Claim 1 is that when the content of Al exceeds 0.004% even being unavoidably included, the composition of the oxides is changed and is highly likely not to function as the nuclei for intragranular ferrite, and thus, the amount of Al is limited to 0.004% or less. As necessary, the upper limit thereof may be 0.003% or 0.002%.

Al is mixed during the refining process of the steel in some cases, and thus, the lower limit thereof is 0.0003%.

The steel according to the embodiment also includes a balance consisting of Fe and unavoidable impurities in addition to the above components. Here, the impurities are components that are mixed on account of various factors in the production process including raw materials such as ore or scrap when steel is produced on an industrial scale and are allowed to be contained within the range such that the components do not exert an adverse influence on the present invention.

The steel plate according to the embodiment may include one or two types or more of Cr, V, Ca, Mg and REM, in addition to the above components. The lower limits of the components do not need to be defined particularly and the lower limits thereof are 0%. In addition, even when the alloy components are intentionally added or mixed as impurities, it is interpreted that the steel is within the scope of the Claims as long as the contents thereof are within the scope of the Claims.

### Cr: 0% to 0.30%

Cr is set to 0.30% or less since Cr deteriorates the CTOD properties of the heat-affected zone. In order to improve the CTOD properties, the upper limit thereof may be 0.20%, 0.15%, 0.10%, or 0.05%. The lower limit of the amount of Cr does not need to be defined particularly, and the lower limit thereof is 0%. However, there is a case that Cr is mixed as an impurity and thus, the lower limit thereof may be 0.001%.

### V: 0% to 0.06%

V is an effective element to improve the strength of the base metal. However, when the amount of V exceeds 0.06%, the CTOD properties are deteriorated, and thus, as a range in which the CTOD properties are not significantly deteriorated, the upper limit is set to 0.06% or less. In order to ensure superior CTOD properties, the upper limit thereof may be 0.04%, 0.02%, or 0.01%. The lower limit of the amount of V does not need to be defined particularly, and the lower limit thereof is 0%. However, even when V is mixed as an impurity, the lower limit thereof may be 0.001%.

### Mg: 0% to 0.0050%

Mg can be included as necessary. When Mg is included, fine Mg-containing oxides are formed and thus, it is effective in γ grain size refinement. However, when the Mg content exceeds 0.0050%, the number of oxides is excessively increased and ductility is reduced. Thus, the upper limit thereof is set to 0.0050%. The upper limit thereof may be limited to 0.0030%, 0.0020%, 0.0010%, or 0.0003%. The lower limit of the Mg content does not need to be defined particularly, and the lower limit thereof is 0%.

The welded steel according to the embodiment may include the following alloy elements for the purpose of further improving the strength and the toughness of the steel itself, or as impurities from auxiliary raw material such as scrap, in addition to the above components.

Ca is mixed as an impurity in some cases and thus, the upper limit thereof may be limited to 0.0010%, 0.0005%, or 0.0003%.

Rare earth metal (REM) is mixed as impurities in some cases and thus, the upper limit thereof may be limited to 0.0010%, 0.0005%, or 0.0003%. Here, the REM is a general term of 17 elements including 15 lanthanoid elements and Y and Sc.

Sb deteriorates the toughness of the HAZ and thus, the upper limit of the Sb content may be 0.03%. In order to improve the toughness of the HAZ, the upper limit of the Sb content may be 0.01%, 0.005%, 0.003%, or 0.001%.

Since As and Sn deteriorate toughness of the HAZ, the upper limits of the As and Sn contents may be 0.02%. As necessary, the upper limits of the As and Sn contents may be 0.005%, 0.003%, or 0.001%. In addition, the lower limits of Ca, REM, Sb, As, and Sn do not need to be defined particularly and the lower limits are 0%.

In addition, to improve the strength and the toughness, each of Pb, Zr, Zn, and W content is set to 0.1% or less, 0.01% or 0.005% or less. The lower limits do not need to be defined particularly and are 0%.

Co is included as an impurity in Ni in some cases. Since Co deteriorates the toughness of the HAZ, the upper limit of the Co content may be 0.05% or 0.002%. The lower limit thereof does not need to be defined particularly, and the lower limit thereof is 0%.

Each of the elements is limited as described above and further, it is necessary that P_{CM} of the following Expression 4 that can be said to be total amount regulation is limited within an appropriate range. The following Expression 4 is a known expression as a weld cracking parameter (P_{CM}). Even when all the elements are within the limitation ranges, the hardenability is insufficient or excessive in a case that all elements are lower limits or all elements are upper limits. In the former case, an increase in thickness and strength cannot be attained and in the latter case, the hardness of the heat-affected zone and MA formation become excessive and thus, it is difficult to ensure toughness. In order to stably ensure the strength with the target thickness of the present invention and stably ensure the toughness of the heat-affected zone, it is necessary to set P_{CM} to 0.18% to 0.23%. ${P}_{CM} = \left[C\right] + \left[Si\right] / 30 + \left[Mn\right] / 20 + \left[Cu\right] / 20 + \left[Ni\right] / 60 + \left[Cr\right] / 20 + \left[Mo\right] / 15 + \left[V\right] / 10 + 5 \left[B\right]$

Here, each of the elements represents the amounts included in the steel by mass%.

Further, it has been found that it is important that the number of oxides having an equivalent circle diameter of 2 µm or more is 20 particles/mm² or less, and the number of Ti oxides included as transformation nuclei in the steel and having an equivalent circle diameter of 0.05 µm to 0.5 µm is 1.0 × 10³ particles/mm² to 1.0 × 10⁵ particles/mm² to satisfy the CTOD properties. When the number of oxides having an equivalent circles diameter of 2 µm or more exceeds 20 particles/mm², the oxides act as a starting point of fracture and the CTOD properties are deteriorated. In addition, when the number of Ti oxides having an equivalent circle diameter of 0.05 µm to 0.5 µm is less than 1.0 × 10³ particles/mm², the number of Ti oxides as nuclei for forming intragranular transformation ferrite is insufficient and when the number of Ti oxides exceeds 1.0 × 10⁵ particles/mm², the Ti oxides act as a starting point of fracture, and in both the cases, the CTOD properties are deteriorated.

It is also necessary to limit the production method to industrially produce a thick high strength steel plate with stability while limiting the components of the steel as described above.

Next, an example of a method of producing an ultrahigh tensile strength steel for welding will be described.

It is preferable that the steel of the present invention is produced industrially by a continuous casting method. The reason is that the solidification cooling rate of molten steel is high and a large amount of fine Ti oxides and Ti nitrides can be formed in a slab. In the method of producing the welded steel according to the embodiment, it is preferable that an average cooling rate at the center portion of the slab to 800°C from around a solidifying point is 5 °C/min or higher. The reason is to obtain oxides having an equivalent circle diameter of 2 µm or more of 20 particles/mm² or less and Ti oxides having an equivalent circle diameter of 0.05 µm to 0.5 µm of 1.0 × 10³ particles/mm² to 1.0 × 10⁵ particles/mm² in the steel. When the cooling rate of the slab is lower than 5 °C/min, fine oxides are hardly obtained and coarse oxides increase. On the other hand, even when the average cooling rate exceeds 50 °C/min, the number of fine Ti oxides does not significantly increase and the cost of production rather increases, and thus, the average cooling rate may be 50 °C/min or lower.

The average cooling rate at the center portion of the slab can be obtained by measuring the cooling rate of the surface of the slab and performing thermal conduction calculation. In addition, the average cooling rate can also be obtained by measuring a casting temperature and an amount of cooling water and performing thermal conduction calculation.

When the slab is rolled, the re-heating temperature thereof is preferably 1000°C to 1100°C. When the re-heating temperature exceeds 1100°C, the Ti oxides are coarsened and an effect of improving deterioration in toughness of the base metal or the toughness of the HAZ cannot be expected. In addition, at a re-heating temperature of lower than 1000°C, rolling reaction force increases and a rolling load increases, and thus, the productivity is impaired.

After the re-heating; production in TMCP is required. First, rolling is performed at a temperature of 950°C or higher under a cumulative reduction of 30% or more. In the rolling in a high temperature region, the grains of heated coarse austenite are sized and refined, and thus, the more the cumulative reduction, the more preferable it is. However, the rolling in a high temperature region is regulated by the thickness of the slab and the subsequent rolling conditions. It is difficult to grasp the rolled structure in a high temperature state, but in the factory or laboratory test of the inventors, when the cumulative reduction is 30% or more and the subsequent rolling-cooling conditions are within an appropriate range, it has been confirmed that the properties are stable.

Next, the rolling is performed under a cumulative reduction of 40% or more at a temperature of 720°C to 950°C and a total cumulative reduction of 60% or more, and the rolling is finished at a temperature of 700°C to 750°C. The temperature regions are mostly austenite non-recrystallization temperature regions. However, since thick material has temperature distribution in a thickness direction and has a high temperature in the vicinity of the thickness center portion, rolling may not be sufficiently performed in the non-recrystallization temperature region. Therefore, the temperature and the cumulative reduction are limited in two stages the in the present invention. The rolling under a cumulative reduction of 40% or more at a temperature of 720°C to 950°C is a minimum required rolling reduction in austenite non-recrystallization by a depth of about 1/4 of the thickness from the surface layers of the front and rear surfaces. Further, the reason for finishing the rolling with a total cumulative reduction of 60% or more at a temperature of 700°C to 750°C is that the rolling is applied to even to the thickness center portion in the austenite non-recrystallization temperature region to a degree that enables structure refinement. In the thickness center portion, a relatively small reduction in the austenite non-recrystallization temperature region is unavoidable, but the structure can be refined to a degree at which satisfactory a balance between strength and toughness can be ensured with a relatively low heating temperature and an appropriate reduction in a high temperature region limited in the present invention. In the rolling conditions deviated from the limitation ranges, it has been experimentally confirmed that the toughness of the thickness center portion is particularly deteriorated.

Further, as for cooling after the rolling, it is necessary to perform cooling to 280°C or lower by starting water cooling within 80 seconds after the rolling is finished. It is preferable that water cooling start rapidly after the rolling. However, it is unavoidable that a certain period of time is required for transportation from an end of a rolling mill to a cooling facility in large real production facilities. Even in this case, the precipitation of ferrite during air cooling until the cooling after the rolling is not preferable in terms of strength, and the ferrite is highly likely to be coarsened due to precipitation in the air cooling, which is not preferable in terms of toughness. Therefore, it is necessary to start water cooling within 80 seconds after the rolling is finished. The water cooling preferably starts within 60 seconds. Since the water cooling is necessarily performed until transformation is completely completed even at the thickness center portion in which a thermal conduction rate is controlled, cooling to 280°C or lower is necessary. Since an accelerated cooling effect at the thickness center portion of the thick material, which is targeted in the present invention, is obtained, it is preferable to perform cooling at a sprayed water density of about 1.2 m³m²/min or more.

After the cooling, tempering has to be performed in a temperature range of 400°C to 550°C. By performing the tempering, the balance between strength and toughness of the base metal are improved and also can be stably controlled with high accuracy. Further, nonuniformity at the time of cooling is alleviated, and thus, an effect of releasing residual stress in the steel is obtained. Also, shape change caused by the nonuniformity and the residual stress at the time of cutting is suppressed. When the tempering is performed at a temperature of lower than 400°C, the effects are reduced and when the tempering is performed at a temperature of higher than 550°C, the strength is significantly reduced and it is difficult to ensure high strength that is targeted in the present invention.

Here, all the aforementioned temperatures are steel surface temperatures.

From the above, in the method of producing the ultrahigh tensile strength steel for welding having excellent weldability and toughness of the heat-affected zone, for example, a steel piece or a cast piece having the steel components described (1) is heated at a temperature of 1000°C to 1100°C, rolling is finished such that the cumulative reduction is 30% or more at a temperature of 950°C or higher, the cumulative reduction is 40% or more at a temperature of 720°C to 950°C, and the cumulative reduction is 60% or more at a temperature of 700°C to 750°C, water cooling is performed within 80 seconds after the rolling is finished to cool the steel to 280°C or lower, and then, further tempering is performed in a temperature range of 400°C to 550°C.

### [Examples]

Hereinafter, the present invention will be described based on Examples and Comparative examples.

Using a converter, continuous casting, and rolling process, a thick steel plate having various kinds of steel components was produced, and the toughness of the base metal and the heat-affected zone was evaluated.

The welding was performed by the submerged arc welding method that is generally used as test welding and multilayer welding was performed with a weld heat input of 4.5 kJ/mm at a K groove so that the weld fusion line (FL) became vertical. As the toughness evaluation of the heat-affected zone, a CTOD test was performed according to American Petroleum Institute (API) standard RP 2Z and British Standard (BS) 7448. Notches were made on the fusion line that is referred to as coarse grain HAZ (CGHAZ) and six pieces were tested at a test temperature of -10°C on each.

In Tables 1-1 to 1-4, the chemical components of the steels are shown and in Tables 2-1 to 2-4, the manufacturing condition, the number of oxides in the steels, the properties of the base metal, the toughness of the heat-affected zone (CTOD properties) are shown. In the steel plates produced in the present invention (invention steels: steel component Nos. 1 to 15 and 29 to 51, and Example Nos. A1 to L2), the yield strength (YS) was 526 MPa to 611 MPa at a depth position of 1/4 of the steel plate and the yield strength was 516 MPa to 594 MPa at a depth position of 1/2 of the steel plate, and the tensile strength (TS) was 616 MPa to 680 MPa at a depth position of 1/4 of the steel plate and the tensile strength was 604 MPa to 656 MPa at a depth position of 1/2 of the steel plate. In the fracture transition (vTrs) test results of the toughness of the base metal, the fracture transition temperatures were -48°C to -81°C at a depth position of 1/4 of the steel plate and the fracture transition temperatures were -40°C to -68°C at a depth position of 1/2 of the steel plate, and the lowest CTOD value at -10°C was 0.29 mm to 0.94 mm, and thus, satisfactory fracture toughness was exhibited. Further, satisfactory weldability was exhibited by the P_{CM} values and the CTOD properties of the invention steels.

On the other hand, in the steel plates of the Comparative examples deviated from the limitation ranges of the present invention (comparative steels: steel component Nos. 16 to 28 and 52 to 62, and Comparative example Nos. a to x), the strength of the base metal was decreased, the toughness of the base metal was deteriorated, or the toughness of the heat-affected zone was deteriorated.

That is, the steel components in Comparative examples a to c, Comparative examples e to o, and Comparative examples q to v were out of the range of the present invention and the above-described mechanical properties were not satisfied. Particularly, since Comparative example f with the steel component No. 21 did not satisfy Ni/Cu > 2.0, cracking occurred at the time of hot rolling and thus the production was difficult. Further, Comparative examples d, w, and x whose steel components are within the range of the present invention but the FB or P_{CM} values are out of the range of the present invention did not satisfy FB ≥ 0.0003%, or the P_{CM} value was not within a range of 0.18% to 0.23%, and thus, the strength of the base metal was decreased or increased, the toughness of the base metal was deteriorated, or the toughness of the heat-affected zone was deteriorated.

### [Industrial Applicability]

According to the present invention, it is possible to provide the ultrahigh tensile strength steel having excellent weldability and toughness of the heat-affected zone at a low cost and also possible to further increase safety while the size of a welded structure such as an offshore structure can be increased.

## Claims

1. A steel plate consisting of, as a chemical composition, by mass%,
C: 0.015% to 0.045%,
Mn: 1.80% to 2.20%,
Cu: 0.40% to 0.70%,
Ni: 0.80% to 1.80%,
Nb: 0.005% to 0.015%,
Mo: 0.05% to 0.25%,
Ti: 0.005% to 0.015%,
B: 0.0004% to 0.0020%,
N: 0.0020% to 0.0060%,
O: 0.0015% to 0.0035%,
Si: 0.01% to 0.40%,
P: 0.008% or less,
S: 0.005% or less,
Al: 0.0003% to 0.004%,
Cr: 0% to 0.30%,
V: 0% to 0.06%,
Mg: 0% to 0.0050%, and
a balance consisting of Fe and unavoidable impurities,
wherein a value expressed by a following Expression 1 is more than 2.0,
a value expressed by a following Expression 2 is 0% or more,
FB expressed by a following Expression 3 is 0.0003% or more,
a P_{CM} value which is a weld cracking parameter expressed by a following Expression 4 is 0.18% to 0.23%,
a Bp expressed by a following Expression 5 is 0.09% to 0.30%, and
a number of oxide grains having an equivalent circle diameter of 2 µm or more is 20 particles/mm² or less and a number of Ti oxides having an equivalent circle diameter of 0.05 µm to 0.5 µm is 1.0 × 10³ particles/mm² to 1.0 × 10⁵ particles/mm² at a thickness center portion of a cross section in a thickness direction, $\left[Ni\right] / \left[Cu\right]$ $\left[N\right] - \left[Ti\right] / 3.4$ $FB = \left[B\right] - 0.77 \times \left(\left[N\right]-0.29\times \left(\left[Ti\right]-2\times \left(\left[O\right]-0.89\times \left[Al\right]\right)\right)\right)$ ${P}_{CM} = \left[C\right] + \left[Si\right] / 30 + \left[Mn\right] / 20 + \left[Cu\right] / 20 + \left[Ni\right] / 60 + \left[Cr\right] / 20 + \left[Mo\right] / 15 + \left[V\right] / 10 + 5 \left[B\right]$ $Bp = \left(884\times \left[C\right]\times \left(1-0.3\times {\left[C\right]}^{2}\right)+294\right) \times FB$ here, [C], [Si], [Mn], [Cu], [Ni], [Cr], [Mo], [V], [Ti], [B], [N], [O], and [Al] represent respectively C, Si, Mn, Cu, Ni, Cr, Mo, V, Ti, B, N, O, and Al contents by mass%, however, when the term of ([O] - 0.89 × [Al]) in the Expression 3 is 0 or less, the term of ([O] - 0.89 × [Al]) in the Expression 3 is set to 0 to calculate the FB, also, when the term of ([Ti] - 2 × ([O] - 0.89 × [Al])) in the Expression 3 is 0 or less, the term of ([Ti] - 2 × ([O] - 0.89 × [Al])) in the Expression 3 is set to 0 to calculate the FB,
further, when the term of ([N] - 0.29 × ([Ti] - 2 × ([O] - 0.89 × [Al]))) in the Expression 3 is 0 or less, the term of ([N] - 0.29 × ([Ti] - 2 × ([O] - 0.89 × [Al]))) in the Expression 3 is set to 0 to calculate the FB, and
still further, when FB ≤ 0, FB = 0.

2. The steel plate according to claim 1, further comprising, as the chemical composition, by mass%,
Si: limited to 0.15% or less.

3. The steel plate according to claim 1 or 2, further comprising, as the chemical composition, by mass%,
Mg: limited to less than 0.0003%.

4. The steel plate according to any one of claims 1 to 3,
wherein a thickness is 50 mm or more and 100 mm or less,
a tensile strength is 600 MPa or more and 700 MPa or less, and
a yield strength is 500 MPa or more and 690 MPa or less.

## Patentansprüche

1. Eine Stahlplatte, bestehend aus, als eine chemische Zusammensetzung, in Massen-%,
C: 0,015% bis 0,045%,
Mn: 1,80% bis 2,20 %,
Cu: 0,40% bis 0,70%,
Ni: 0,80% bis 1,80%,
Nb: 0,005% bis 0,015%,
Mo: 0,05% bis 0,25%,
Ti: 0,005% bis 0,015%,
B: 0,0004% bis 0,0020%,
N: 0,0020% bis 0,0060%,
O: 0,0015% bis 0,0035%,
Si: 0,01% bis 0,40%,
P: 0,008% oder weniger,
S: 0,005% oder weniger,
Al: 0,0003% bis 0,004%,
Cr: 0% bis 0,30%,
V: 0% bis 0,06%,
Mg: 0% bis 0,0050% und
einem Rest bestehend aus Fe und unvermeidbaren Verunreinigungen,
wobei ein Wert, ausgedrückt durch einen folgenden Ausdruck 1, mehr als 2,0 beträgt,
ein Wert, ausgedrückt durch einen folgenden Ausdruck 2, 0% oder mehr beträgt,
FB, ausgedrückt durch einen folgenden Ausdruck 3, 0,0003% oder mehr beträgt,
ein P_{CM}-Wert, welcher ein Parameter für Schweissnahtrissbildung ist, ausgedrückt durch den folgenden Ausdruck 4, 0,18% bis 0,23% beträgt,
ein Bp, ausgedrückt durch den folgenden Ausdruck 5, 0,09 bis 0,30% beträgt und
eine Anzahl an Oxidkörnern mit einem äquivalenten Kreisdurchmesser von 2 µm oder mehr 20 Teilchen/mm² oder weniger und eine Anzahl an Ti-Oxiden mit einem
äquivalenten Kreisdurchmesser von 0,05 µm bis 0,5 µm 1,0 x 10³ Teilchen/mm² bis 1,0 x 10⁵ Teilchen/mm² in einem mittleren Bereich der Dicke in einem Querschnitt entlang einer Dickenrichtung beträgt, $\left[Ni\right] / \left[Cu\right]$ $\left[N\right] - \left[Ti\right] / 3 , 4$ $FB = \left[B\right] - 0 , 77 \times \left(\left[N\right]-0,29\times \left(\left[Ti\right]-2\times \left(\left[O\right]-0,89\times \left[A1\right]\right)\right)\right)$ ${P}_{CM} = \left[C\right] + \left[Si\right] / 30 + \left[Mn\right] / 20 + \left[Cu\right] / 20 + \left[Ni\right] / 60 + \left[Cr\right] / 20 + \left[Mo\right] / 15 + \left[V\right] / 10 + 5 \left[B\right]$ $Bp = \left(884\times \left[C\right]\times \left(1-0,3\times {\left[C\right]}^{2}\right)+294\right) \times FB$ hier stellen [C], [Si], [Mn], [Cu], [Ni], [Cr], [Mo], [V], [Ti], [B], [N], [O], und [Al] jeweils C, Si, Mn, Cu, Ni, Cr, Mo, V, Ti, B, N, O und Al-Gehalte in Massen-% dar,
wenn jedoch der Term ([O] - 0,89 × [Al]) im Ausdruck 3 0 oder weniger beträgt, wird der Term ([O] - 0,89 × [Al]) im Ausdruck 3 auf 0 festgelegt, um den FB zu berechnen, ebenso, wenn der Term ([Ti] - 2 × ([O] - 0,89 × [Al])) im Ausdruck 3 0 oder weniger beträgt, wird der Term ([Ti] - 2 × ([O] - 0,89 × [Al])) im Ausdruck 3 auf 0 festgelegt, um den FB zu berechnen,
ferner, wenn der Term ([N] - 0,29 × ([Ti] - 2 × ([O] - 0,89 × [Al]))) im Ausdruck 3 0 oder weniger beträgt, wird der Term ([N] - 0,29 x ([Ti] - 2 × ([O] - 0,89 × [Al]))) im Ausdruck 3 auf 0 festgelegt, um den FB zu berechnen, und noch ferner, wenn FB ≤ 0, FB=0.

2. Die Stahlplatte gemäß Anspruch 1, ferner umfassend, als chemische Zusammensetzung, in Massen-%,
Si: begrenzt auf 0,15% oder weniger.

3. Die Stahlplatte gemäß Anspruch 1 oder 2, ferner umfassend, als chemische Zusammensetzung, in Massen-%,
Mg: begrenzt auf weniger als 0,0003%.

4. Die Stahlplatte gemäß einem der Ansprüche 1 bis 3,
wobei eine Dicke 50 mm oder mehr und 100 mm oder weniger beträgt,
eine Zugfestigkeit 600 MPa oder mehr und 700 MPa oder weniger beträgt und
eine Streckgrenze 500 MPa oder mehr und 690 MPa oder weniger beträgt.

## Revendications

1. Plaque d'acier constituée de, comme une composition chimique, en % en masse,
C : 0,015 % à 0,045 %,
Mn : 1,80 % à 2,20 %,
Cu : 0,40 % à 0,70 %,
Ni : 0,80 % à 1,80 %,
Nb : 0,005 % à 0,015 %,
Mo : 0,05 % à 0,25 %,
Ti : 0,005 % à 0,015 %,
B : 0,0004 % à 0,0020 %,
N : 0,0020 % à 0,0060 %,
O : 0,0015 % à 0,0035 %,
Si : 0,01 % à 0,40 %,
P : 0,008 % ou moins,
S : 0,005 % ou moins,
Al : 0,0003 % à 0,004 %,
Cr : 0 % à 0,30 %,
V : 0 % à 0,06 %,
Mg : 0 % à 0,0050 %, et
un reste constitué de Fe et d'impuretés inévitables,
dans laquelle une valeur exprimée par une expression 1 suivante est supérieure à 2,0,
une valeur qui exprimée par une expression 2 suivante est de 0 % ou supérieure,
FB exprimé par une expression 3 suivante est de 0,0003 % ou supérieur,
une valeur P_{CM} est un paramètre de craquage de soudure exprimée par une expression 4 suivante est de 0,18 % à 0,23 %,
un Bp exprimé par une expression 5 suivante est de 0,09 % à 0,30 %, et
un nombre de grains d'oxyde présentant un diamètre de cercle équivalent de 2 µm ou supérieur est de 20 particules/mm² ou inférieur et un nombre d'oxydes de Ti ayant un diamètre de cercle équivalent de 0,05 µm à 0,5 µm est de 1,0 x 10³ particules/mm² à 1,0 x 10⁵ particules/mm² dans une portion centrale d'épaisseur d'une section transversale dans une direction d'épaisseur, $\left[Ni\right] / \left[Cu\right]$ $\left[N\right] - \left[Ti\right] / 3 , 4$ $FB = \left[B\right] - 0 , 77 \times \left(\left[N\right]-0,29\times \left(\left[Ti\right]-2\times \left(\left[O\right]-0,89\times \left[Al\right]\right)\right)\right)$ ${P}_{CM} = \left[C\right] + \left[Si\right] / 30 + \left[Mn\right] / 20 + \left[Cu\right] / 20 + \left[Ni\right] / 60 + \left[Cr\right] / 20 + \left[Mo\right] / 15 + \left[V\right] / 10 + 5 \left[B\right]$ $Bp = \left(884\times \left[C\right]\times \left(1-0,3\times {\left[C\right]}^{2}\right)+294\right) \times FB$ ici, [C], [Si], [Mn], [Cu], [Ni], [Cr], [Mo], [V], [Ti], [B], [N], [O], et [Al représentent respectivement les teneurs en C, Si, Mn, Cu, Ni, Cr, Mo, V, Ti, B, N, O et Al en % en masse,
cependant, lorsque le terme de ([O]-0,89 x [Al]) dans l'expression 3 est inférieur ou égal à 0, le terme de ([O]-0,89 x [Al]) dans l'expression 3 est fixé à 0 pour calculer le FB,
également, lorsque le terme de ([Ti]-2 x ([O]-0,89 x [Al])) dans l'expression 3 est inférieur ou égal à 0, le terme de ([Ti]-2 x ([O]-0,89 x [Al])) dans l'expression 3 est fixé à 0 pour calculer le FB,
de plus, lorsque le terme de ([N] - 0,29 x ([Ti] - 2 x ([O] - 0,89 x [Al]))) dans l'expression 3 est inférieur ou égal à 0, le terme de ([N] - 0,29 x ([Ti] - 2 x ([O] - 0,89 x [Al]))) dans l'expression 3 est fixé à 0 pour calculer le FB et encore plus, lorsque FB ≤ 0, FB = 0.

2. Plaque d'acier selon la revendication 1, comprenant de plus, comme la composition chimique, en % en masse,
Si : limité à 0,15 % ou inférieur.

3. Plaque d'acier selon la revendication 1 ou 2, comprenant de plus, comme la composition chimique, en % en masse,
Mg : limité à moins de 0,0003 %.

4. Plaque d'acier selon l'une quelconque des revendications 1 à 3,
dans laquelle une épaisseur est de 50 mm ou supérieure et de 100 mm ou inférieure,
une résistance à la traction est de 600 MPa ou supérieure et de 700 MPa ou inférieure, et
une limite d'élasticité est de 500 MPa ou supérieure et de 690 MPa ou inférieure.
